

Nov. 28, 1939.

M. HERBST ET AL

2,181,485

GELATIN RELIEF

Filed May 11, 1938

Fig. 3



Fig. 1.



By Their Attorneys

Max Herbst  
Walter Frankenburger

Harry and Joslin

## UNITED STATES PATENT OFFICE

2,181,485

## GELATIN RELIEF

Max Herbet, Mannheim-Rheinau, and Walter Frankenburger, Ludwigshafen, Germany, assignor, by mesme assignments, to Agfa Ansco Corporation, Binghamton, N. Y., a corporation of Delaware

Application May 11, 1938, Serial No. 207,226  
In Germany May 13, 1937

8 Claims. (Cl. 95—5.6)

The present invention relates to gelatin reliefs for printing.

It is known to produce gelatin reliefs for printing by using silver halide layers which are dyed 5 complementarily to their spectral sensitivities (cf. U. S. Patent No. 2,061,230) dated November 17, 1936.

It is an object of the present invention to provide a process by which the effect desired by this 10 dyeing, namely a soft gradation of the relief, is produced by dyeing the sensitized emulsion complementarily only to a part of the sensitizing region. By "sensitizing region" is to be understood the region of the wave lengths of the spectral 15 sensitivity diminished by that of the natural sensitivity of the non-sensitized emulsion, that is to say that spectral region in which the sensitivity natural to the non-sensitized silver halide emulsion is increased by the sensitizing. It follows that, for example, yellow or orange dyeings, such as are used in the duplicating films and the like or for damping the blue sensitivity, that is to say the natural sensitivity of the silver halide, are not within this invention.

20 Further objects of the invention will appear from the following description.

Reference is made to the accompanying diagrams 1 to 4 which illustrate the invention for different spectral regions.

25 The advantage of a dyeing which is only in part complementary consists especially in an essential increase of general sensitivity. Any dyeing which absorbs light in the region of the sensitivity of the silver halide to light diminishes 30 the sensitivity on purely optical grounds; by a narrow spectral limitation of the dyeing, however, this loss of sensitivity is diminished. On the other hand, since it has been found that wholly undyed silver halide layers yield objectionably 35 hard reliefs, it was unexpected that a dyeing which absorbs only a portion of the sensitizing region should suffice to produce a satisfactory gradation especially since for orthochromatically or panchromatically sensitized layers yellow or 40 orange coloring, the absorption of which embraces only violet, blue and green of short wave length, that is to say is only complementary to the natural sensitivity of the silver halide, is practically ineffective in respect of improving gradation of the etching.

45 It is advantageous to use such colorings as have an increasing absorption capacity towards the long wave lengths starting from 540 m $\mu$  or still longer, since it is particularly the light of the

long wave length that produces gradation for etched reliefs.

The following examples illustrate the invention but they are not intended to limit it thereto:

5 1. A silver bromide emulsion, the sensitivity curve of which towards the long wave lengths extends to 480 m $\mu$  (A in Figure 1) is sensitized orthochromatically so that its sensitivity now extends to 600 m $\mu$  (as indicated at B). The region between A and B corresponds with the sensitizing region. In order to make this sensitized emulsion suitable for etched reliefs, it is mixed with a blue-green dye, for instance, "Fanalbremerblau" (cf. Schultz, Farbstofftabellen, 7th edit., vol. I, 1931, No. 826) the light absorption curve 10 of which begins at 530 m $\mu$  (as indicated at C) and increases towards the long wave lengths.

15 2. A panchromatically sensitized silver halide emulsion the sensitivity of which is represented by the curve 1 shown in Figure 2 is made useful 20 for etched reliefs by mixing it with a finely dispersed colorless solid substance of which the main part has a particle diameter not exceeding 1  $\mu$  which substance does not influence the silver halide and is insoluble in the photographic treating baths, and with a blue-green dyestuff, (for instance, ultramarine) the light absorption capacity of which embraces the region between 570 25 and 700 m $\mu$  as indicated by curve 2.

30 3. In order to make a sensitized silver bromide emulsion, the sensitivity curve of which towards the long wave lengths extends to 520 m $\mu$  (AB is the sensitizing region, cf. Figure 3), suitable for producing etched reliefs, the emulsion is mixed with a dyestuff, for instance, "Alizarinrotlack" 35 or "Fanalrosa B" (cf. Schultz, Farbstofftabellen, 7th edit., vol. I, 1931, No. 865) the luminous absorption curve of which starts from 500 m $\mu$  (C) and extends to any point above 520 m $\mu$ .

40 4. An orthochromatically sensitized silver halide gelatin emulsion the sensitivity curve of which extends to 620 m $\mu$  (sensitizing region AB, cf. Figure 4) is colored with a dye (cinnabar, for instance) the luminous absorption capacity of which begins in the long wave range at 600 m $\mu$  45 (G) and extends towards the short wave lengths up to any points, for instance 500 m $\mu$  (C), 420 m $\mu$  (E) or still further (F).

45 For obtaining gelatin reliefs for printing the emulsion layers as above described are exposed 50 to light, developed by the usual method without tanning and fixed. The relief is produced by etching with a solution of hydrogen peroxide (cf. Wall, The History of Three-Color Photography, 1925, page 357).

We claim:

1. A process of producing a gelatin relief for printing which comprises incorporating in a silver halide gelatin emulsion a solid substance of which the main part has a particle diameter not exceeding  $1 \mu$  which substance does not affect the silver halide and is insoluble in the photographic treating baths, sensitizing said silver halide emulsion for a spectral region different from its initial sensitivity, dyeing said silver halide emulsion in a color complementary only to a part of said spectral region, casting said emulsion on a support to form a layer, producing a latent image in said layer, developing said image to a silver picture, and etching said layer to form a relief.
2. A process of producing a gelatin relief for printing which comprises incorporating in a silver halide gelatin emulsion a solid substance of which the main part has a particle diameter not exceeding  $1 \mu$  which substance does not affect the silver halide and is insoluble in the photographic treating baths, sensitizing said silver halide emulsion panchromatically, mixing said silver halide emulsion with a dyestuff the light absorption curve of which embraces the region between 570 and 700  $m\mu$ , casting said emulsion on a support to form a layer, producing a latent image in said layer, developing said image to a silver picture, and etching said layer to form a relief.
3. A process of producing a gelatin relief for printing which comprises incorporating in a silver halide gelatin emulsion a solid substance of which the main part has a particle diameter not exceeding  $1 \mu$  which substance does not affect the silver halide and is insoluble in the photographic treating baths, sensitizing said silver halide emulsion orthochromatically, mixing said silver halide emulsion with a dyestuff the light absorption curve of which begins at 530  $m\mu$  and increases towards the long wave lengths, casting said emulsion on a support to form a layer, producing a latent image in said layer, developing said image to a silver picture, and etching said layer to form a relief.
4. A process of producing a gelatin relief for printing which comprises incorporating in a silver halide gelatin emulsion a solid substance of which the main part has a particle diameter not exceeding  $1 \mu$  which substance does not affect the silver halide and is insoluble in the photographic treating baths, sensitizing said silver halide emulsion orthochromatically, mixing said silver halide emulsion with a dyestuff the light absorption curve of which begins in the long-wave region at 600  $m\mu$  and extends towards the short wave lengths up to any point.
5. A photographic material which comprises a support and attached to said support a silver halide gelatin emulsion layer containing a solid substance of which the main part has a particle diameter not exceeding  $1 \mu$  which substance does not affect the silver halide and is insoluble in the photographic treating baths, said emulsion layer being sensitized for a spectral region different from its initial sensitivity and being colored only with a dyestuff of a color complementary only to a part of said spectral region.
6. A photographic material which comprises a support and attached to said support a silver halide gelatin emulsion layer containing a solid substance of which the main part has a particle diameter not exceeding  $1 \mu$  which substance does not affect the silver halide and is insoluble in the photographic treating baths, said emulsion layer being sensitized panchromatically and being colored only with a dyestuff the light absorption curve of which embraces the region between 570 and 700  $m\mu$ .
7. A photographic material which comprises a support and attached to said support a silver halide gelatin emulsion layer containing a solid substance of which the main part has a particle diameter not exceeding  $1 \mu$  which substance does not affect the silver halide and is insoluble in the photographic treating baths, said emulsion layer being sensitized orthochromatically and being colored only with a dyestuff the light absorption curve of which begins at 530  $m\mu$  and increases towards the long wave lengths.
8. A photographic material which comprises a support and attached to said support a silver halide gelatin emulsion layer containing a solid substance of which the main part has a particle diameter not exceeding  $1 \mu$  which substance does not affect the silver halide and is insoluble in the photographic treating baths, said emulsion layer being sensitized orthochromatically and being colored only with a dyestuff the light absorption curve of which begins in the long-wave region at 600  $m\mu$  and extends towards the short wave lengths up to any point.

MAX HERBST.  
WALTER FRANKENBURGER.